

115  
Oct. 16, 1956

M. H. EDSON  
AN ASPHALT, A PROCESS OF MAKING IT AND  
AN ENAMEL MADE THEREWITH  
Filed Nov. 28, 1952

2,767,102

SUBSTITUTE FOR MISSING XR



Murray H. Edson Inventor  
By W.O. Heilman Attorney

1

2,767,102

## AN ASPHALT, A PROCESS OF MAKING IT AND AN ENAMEL MADE THEREWITH

Murray H. Edson, Rahway, N. J., assignor to Esso Research and Engineering Company, a corporation of Delaware

Application November 28, 1952, Serial No. 322,919

4 Claims. (Cl. 106—281)

The objects of this invention are a novel asphaltic composition, a process of making it and an improved enamel composition particularly adapted for use in the protective coating of pipelines. In this application of the invention, the enamel constitutes a tar obtained by air-blowing a vacuum reduced, thermally cracked feed stock constituting catalytic cycle oil in combination with inorganic fillers.

The present invention includes an improved process for obtaining a novel asphalt. The process requires the catalytic cracking of a petroleum oil feed stock to provide a catalytic cycle oil. This cycle oil, after removal of any entrained catalyst, is subjected to thermal cracking and a thermal tar is obtained by vac-distilling the lighter constituents from the thermally cracked products. This thermal tar is then oxidized, as by blowing air through the tar, so as to provide the final asphalt product. This asphalt possesses an unique combination of physical properties. In general, the asphalt will possess a penetration (ASTM D-5) of zero at 77° F./100 g./5" and less than 6 at 115° F./100 g./5", and a softening point of about 160° to 210° F. Enamels made from this asphalt are characterized by shatter resistance, slip resistance, hardness, and low application temperature.

At the present time a variety of processes are known for obtaining asphalts from crude petroleum oils. For example, residual petroleum oils may be oxidized by air-blowing to provide asphalts. Again, residual oils may be subjected to vacuum distillation so as to obtain asphalts. A variety of treating re-agents may also be employed to convert a residual oil to an asphalt. Each of the processes which may be employed for asphalt manufacture result in asphalts having a particular interrelation of physical properties. Thus, for example, asphalts obtained by the air-blowing of residual oils are characterized by high softening points, low temperature susceptibility, and high values of penetration. Asphalts obtained from the other processes indicated, possess somewhat different properties in these and other respects.

In order to obtain an asphalt having desirable properties for a particular application, it becomes valuable to develop unusual combinations of asphaltic properties. For example, in using an asphalt for a protective coating as in the enameling of a pipeline, it is important to obtain an asphalt having a high shatter resistance so as to resist fracture due to back-filling or abrasion of the pipeline. Such an asphalt should also have sufficient hardness to resist penetration by rocks, should have a low application temperature to facilitate field usage, a flash point above the application temperature, good "sloughing" characteristics to prevent slipping on the pipeline while cooling, and should not be susceptible to low temperature cracking. In general, presently known asphalts do not have the requisite combination of properties and are par-

2

ticularly deficient in requiring too high a temperature of application and they do not have sufficient hardness.

The present invention is therefore concerned with a new asphalt manufacturing process of a character to provide a novel asphalt having the unusual combination of physical properties referred to. The purpose is primarily to provide an asphalt uniquely qualified for use in pipeline enamels. In accordance with these objectives, it has been found that a new type of asphalt may be obtained by a particular processing sequence. Essentially, the required processing steps concern the catalytic cracking of a heavy boiling fraction of a crude petroleum oil. The heaviest boiling fraction of the catalytically cracked gas oil is then subjected to a thermal cracking operation. Again, the heaviest boiling fraction obtained from the thermal cracking operation is employed and this fraction is subjected to distillation and air-blowing to provide the final asphalt. It is presently believed that the unusual asphalt properties characteristic of the final product are attributable to the chemical composition of the asphalt as a consequence of the treating steps. Thus, it is known that unlike asphalts obtained from other processes, the asphalt of this invention is characterized by a predominance of aromatic hydrocarbons boiling above about 700° F. The asphalts of this invention contain more than 95% of aromatic hydrocarbons. Thus, due to this unique chemical composition of the asphalts, unusual asphaltic properties are appreciated.

In the preferred form of this invention, an asphalt of the character described is admixed with an inorganic filler such as slate flour and mica to provide an enamel. Both the slate flour and mica are employed in finely powdered form. The slate flour preferably constitutes a powder of which 95% will pass through a 325 mesh screen, while 90% of the mica will pass through a 40 mesh screen and not more than 30% through a 100 mesh screen. While varying proportions of mica and slate may be used, it is particularly preferred to use about 20 to 40% of the slate flour and about 5 to 20% of mica admixed with the asphalt. As will be shown, an enamel constituting the particular asphalt of this invention in combination with the slate and mica flour possesses particularly desirable properties for pipeline enameling applications. It is to be understood however, that other fillers such as sand, clay, rock, etc., may be used in powdered form in place of the slate and mica flour.

In order to fully disclose the nature of this invention, reference will be made to the accompanying drawing which diagrammatically illustrates the overall process for obtaining the compositions of this invention. In this drawing, a crude distillation zone 1 is depicted. A crude petroleum oil may be introduced to zone 1 through line 2. The distillation operation is conducted to permit removal of volatile fractions overhead through line 3 and of heavier boiling products such as gasoline, kerosene and heating oils through side stream withdrawals 4, 5, 6, and so on. The heavier boiling fractions having initial boiling ranges of from 800° to 1100° F. and higher are withdrawn as a side stream product through line 7. Residual oil fractions are withdrawn through line 8. It is particularly contemplated that in the practice of this invention, distillation zone 1 be of such a nature as to provide a higher boiling fraction boiling in the range of about 700° to 1100° F., preferably as obtained by vacuum distillation operations. Alternatively, residual oil fractions may be employed. The fraction selected is conducted to a catalytic cracking zone identified by the

rectangle 9. The cracking operation to be conducted in zone 9 is of any desired type employing a catalyst such as modified natural or synthetic clay or gel type catalysts. Examples of these are montmorillonite clays, silica-alumina, silica-magnesia composites, and other conventional cracking catalysts. The operation may be of a continuous or batch nature employing fixed beds, moving beds, fluidized, or suspensoid systems. The heat required for cracking may be supplied as preheat or processed materials and/or as the sensible heat of exothermically regenerated catalyst or in any other conventional manner. The cracking is carried out at temperatures of about 800° to 1000° F., and pressures of about atmospheric to 25 p. s. i. g. or higher. The total cracked products are removed from cracking zone 9 and are conducted to a product fractionator 10. Fractionator 10 is operated to remove lighter fractions of the cracked products through overhead 11, side streams 12, 13, and so on. A bottoms product is obtained from fractionator 10 which may be removed through line 14. In the event the cracking operation conducted in zone 9 was of a fluidized nature, the material withdrawn through line 14 will contain a small percentage of catalyst particles carried over from zone 9. In this case, it is necessary to pass the product stream of line 14 to a settler 15 or otherwise to process the stream to permit separation of the liquid hydrocarbon product from the catalyst. Thus, a clarified hydrocarbon stream is removed from zone 15 through line 16. For the purposes of this invention, the bottoms product of fractionator 10, corresponding to the stream of lines 14 or 16, boils in the range of about 700° to 1100° F. The stream of line 16 is generally called "cycle oil." As the name suggests, cycle oil is generally recycled to the cracking zone, as heretofore virtually no other use has been found for this oil. However, it should be appreciated that return of cycle oil to the cracking operation is not particularly desirable. Cycle oil is refractory in nature and constitutes a very poor cracking feed, causing substantial deposition of carbon and coke on the catalyst employed during cracking. As will be appreciated therefore, it is one of the features of this invention to employ cycle oil so as to prevent recycling to a cracking operation and so as to provide valuable products.

As the conduct of the process as described heretofore is well known to the art, no further description of this phase of the process is considered necessary. The cycle oil of line 16 derived as indicated is then conducted to a thermal cracking zone 20. Zone 20 is employed to thermally crack the cycle oil in the conventional manner. Thus, for example, the thermal cracking zone may constitute a fired coil subjecting the cycle oil passed through to a temperature in the range between 850° and 1200° F., and to a pressure of about 300 to 1000 lbs. per square inch. The preferred thermal cracking conditions employ temperatures of about 900° to 1000° F., pressures of about 650 to 750 p. s. i., and a residence time of about 3 to 6 seconds. The thermal cracking is ordinarily conducted in accordance with this invention to secure a conversion of about 24 to 31% for once-through and 15 to 20% for recycle operations of the heavy boiling feed to constituents boiling below the initial boiling point of the feed.

The total products of the thermal cracking operation are then passed to a distillation zone 31 operated at sub-atmospheric pressures of about 2 to 20 mm. Hg absolute. By introducing the thermally cracked products to this flash zone at a temperature of about 550° to 600° F., lighter thermally cracked constituents are flashed or vaporized and are removed overhead through line 32 of flash zone 31. This distillation operation should be conducted to permit removal as a bottoms product through line 33 of a heavy material having a softening point of 140° to 190° F., a specific gravity at 60° F., of 1.0 to 1.2, and a flash point above 450° F. If desired, the total

products of the thermal cracking operation can be subjected to distillation at atmospheric or higher pressure to remove light fractions prior to the vacuum reduction step.

5 The bottoms product withdrawn from flashing zone 31 is then conducted to an oxidation zone 34 wherein the material is oxidized to a desirable softening point. For this purpose air may be brought into zone 34 through line 35 so as to provide about 30 to 60 cu. ft. of air per minute per ton of asphalt. The air-blowing may be conducted at atmospheric pressures and at temperatures of about 400° F. to 600° F. To secure the objectives of this invention, it is essential that the air-blowing be conducted to secure asphaltic material having a softening point of about 160° to 210° F., preferably 190° to 200° F. Either before or after the air-blowing step, a suitable filler is added to the asphalt to secure the final enamel composition. Preferably the filler is added to the asphalt before air-blowing so that the air will mix and incorporate the filler in the asphalt. Thus, the filler may be introduced directly into the oxidation zone through hopper 36 prior to or during air introduction. The final enamel product may then be withdrawn from zone 34 through line 37 after the oxidation has been completed.

10 In order to demonstrate the unique properties of the composition of this invention, the following data is given showing the properties of a representative enamel prepared in accordance with this invention. The enamel referred to composed 60% of an asphalt derived as illustrated in the drawing, 30% of slate flour sufficiently fine to pass through a 325 mesh sieve, and 10% of mica flour having a particle size such that 90% passed through a 40 mesh screen. Inspections of this enamel are given in Table I. For comparative purposes, the properties of the base asphalt are also given in this table.

Table I

| Enamel                                                    |         |       |         |
|-----------------------------------------------------------|---------|-------|---------|
| Bituminous Base                                           | percent | 100   | 60      |
| Slate Flour through 325 Mesh                              | do      | 0     | 30      |
| Mica Flour                                                | do      | 0     | 10      |
| Specific Gravity at 60° F.                                |         | 1.132 | 1.531   |
| Flash (COC), °F.                                          |         | 535   | 530     |
| Softening Point, (R. & B.), °F.                           |         | 192   | 208     |
| Penetration 77°/100 g./5"                                 |         | 0     | 0       |
| Penetration 100°/100 g./5"                                |         | 0     | 0       |
| Penetration 115°/100 g./5"                                |         | 3     | 1       |
| Penetration 135°/100 g./5"                                |         | 21    | 15      |
| Soluble in CS <sub>2</sub> , Wt. Percent                  |         | 99.9  | 60.0    |
| Soluble in Varsol, Wt. Percent                            |         |       | 47.2    |
| Ash, Percent (ASTM D-482)                                 |         |       | 37.4    |
| Temperature for 2 Poises Vis., °F.                        |         | 338   | 435     |
| Temperature for 18 Poises Vis., °F.                       |         | 285   | 332     |
| Shatter Test—No. of grams for one-blown failure at 77° F. |         |       | 28      |
| Slip Test (160° F., 45°, 2 hrs.) inches                   |         |       | 0.062   |
| Chill Test, Failure at °F.                                |         |       | <32 >20 |
| Settling Test, 5 Hrs./400° F. Ratio: Ash Btm./Ash Orig.   |         |       | 1.31    |
| Hardness Index, 77° F. <sup>1</sup>                       |         | 107   | 177     |

<sup>1</sup> Hardness index defined as "yield point" determined by successive penetration-time relationship.

60 This data indicates that the enamel of this invention has excellent properties for pipeline applications. The flash point, shatter resistance, hardness, application temperature possible, and low temperature characteristics, all qualify the enamel for this application.

65 Referring now to Table II, data is given comparing the enamel of this invention to conventional enamels. In Table II five columns are shown giving the properties of five different pipeline enamels. The first column shows the properties of the enamel identified in Table I. The second column shows the properties of a similar enamel which contains only slate flour as a filler. Column 3 shows the properties of a conventional enamel not made in accordance with this invention constituting 40% of slate flour admixed with a noncatalytically cracked thermally cracked tar which has been fire and steam reduced to a 180° to 190° F. softening point. Finally, the last two columns of Table II show the properties of enamels prepared by mixing slate flour with cold tar.

Table II

|                                                    | Air Blowing a Vacuum Reduced 160° F. Softening Point, Catalytically Cracked Thermally Cracked Tar With Slate Flour and Mica | Air Blowing a Vacuum Reduced 140° F. Softening Point, Catalytically Cracked Thermally Cracked Tar With 40% Slate Flour | Mixing 40% Slate Flour With Fire and Steam Reduced 180/190° F. Softening Point, Non-Catalytically Cracked Thermally Cracked Tar | 30% of Slate Flour Mixed With Coal Tar |
|----------------------------------------------------|-----------------------------------------------------------------------------------------------------------------------------|------------------------------------------------------------------------------------------------------------------------|---------------------------------------------------------------------------------------------------------------------------------|----------------------------------------|
| Hardness Index.....                                | 177                                                                                                                         | 44                                                                                                                     | 56                                                                                                                              | 160                                    |
| Shatter Resistance (Grams for 1 blow failure)..... | 28                                                                                                                          | 19                                                                                                                     | 8                                                                                                                               | 81                                     |
| Temp. for 2 poise Vis., ° F.....                   | 435                                                                                                                         | 399                                                                                                                    | 455                                                                                                                             | 373                                    |
| Temp. for 18 Poise Vis., ° F.....                  | 332                                                                                                                         | 308                                                                                                                    | 351                                                                                                                             | 303                                    |
| Slip, inches @ 160° F., 2 hrs. 45°.....            | 1/16                                                                                                                        | 1/6                                                                                                                    | 1/2                                                                                                                             | 2                                      |
| Settling (Ash bottom/Ash Orig.).....               | 1.31                                                                                                                        | 1.57                                                                                                                   | 1.47                                                                                                                            | 2.43                                   |
| Chill, failure @ ° F.....                          | <32                                                                                                                         | >20                                                                                                                    | <32                                                                                                                             | >20                                    |
| Softening Point (R. & B.) ° F.....                 | 208                                                                                                                         | 192                                                                                                                    | 205                                                                                                                             | 200                                    |
| Specific Gravity @ 60° F.....                      | 1.531                                                                                                                       | 1.515                                                                                                                  | 1.494                                                                                                                           | 1.402                                  |
| Flash, COC, ° F.....                               | 630                                                                                                                         | 590                                                                                                                    | 555                                                                                                                             | 465                                    |
| Penetration 77°/100 g./5'.....                     | 0                                                                                                                           | 0                                                                                                                      | 0                                                                                                                               | 0                                      |
| Penetration 100°/100 g./5'.....                    | 0                                                                                                                           | 0                                                                                                                      | 4                                                                                                                               | 0                                      |
| Penetration 115°/100 g./5'.....                    | 1                                                                                                                           | 4                                                                                                                      | 7                                                                                                                               | 1                                      |
| Penetration 135°/100 g./5'.....                    | 15                                                                                                                          | 31                                                                                                                     | 22                                                                                                                              | 13                                     |
| Ash, Wt. Percent (ASTM D-482).....                 | 37.4                                                                                                                        | 38.4                                                                                                                   | 40.2                                                                                                                            | 26.3                                   |
|                                                    |                                                                                                                             |                                                                                                                        |                                                                                                                                 | 27.9                                   |

As shown by the data of Table II, the preferred enamel composition of this invention characterized in column 1 of the table is superior to all other enamels shown in the table. The superiority is established by considering the properties of hardness, shatter resistance, slip characteristics, settling characteristics, and the application temperature. The enamel of column 2, which is an enamel within the scope of this invention, exhibits good properties and is superior to the similar enamel of column 3, which, however, was not vacuum reduced. The superiority of vacuum reduction as compared to fire and steam reduction is shown by comparing the properties of shatter resistance, slip characteristics, flash point, and application temperature. This data therefore establishes the desirable properties of the enamels of this invention compared to conventional enamels. Furthermore, the data shows the particular benefit obtained in preparing the enamel of this invention by vacuum reducing the catalytically cracked-thermally cracked tar to the desired softening point.

What is claimed is:

1. An asphalt material derived by catalytic cracking of a heavy boiling fraction of a petroleum crude oil to provide a catalytic cycle oil, said cycle oil being thermally cracked and vacuum reduced to provide a tar, said tar thereafter being air-blown to provide an asphalt containing at least about 95% of aromatic hydrocarbons and having a softening point of about 160° F. to 210° F.

2. An asphalt enamel including about 60% of an

asphalt derived from an asphalt material derived by catalytic cracking of a heavy boiling fraction of a petroleum crude oil to provide a catalytic cycle oil, said cycle oil being thermally cracked and vacuum reduced to provide a tar, said tar thereafter being air-blown to provide an asphalt containing at least about 95% of aromatic hydrocarbons and having a softening point of about 160° to 200° F., in combination with about 40% of a filler.

3. The enamel defined by claim 2 in which the said filler is a mixture of slate flour and mica.

4. A process for preparing an improved asphalt for enamel compositions comprising catalytically cracking a heavy boiling fraction of a petroleum crude oil to provide a catalytic cycle oil, thermally cracking said catalytic cycle oil and segregating a tar fraction, and vacuum reducing said tar fraction and oxidizing the tar to provide an asphalt containing at least about 95% of aromatic hydrocarbons and having a softening point of about 160° to 210° F.

#### References Cited in the file of this patent

| UNITED STATES PATENTS |                |                |
|-----------------------|----------------|----------------|
| 2,096,876             | Ditzer         | Oct. 26, 1937  |
| 2,220,714             | Hersberger     | Nov. 5, 1940   |
| 2,305,440             | Noel           | Dec. 15, 1942  |
| 50 2,383,701          | Becker et al.  | Aug. 28, 1945  |
| 2,384,671             | Fratis         | Sept. 11, 1945 |
| 2,608,470             | Helmers et al. | Aug. 26, 1952  |